

3,738,981

**TEXTILE TREATING COMPOSITIONS, PROCESS OF  
TREATING TEXTILES AND TEXTILE ARTICLES**

Kenneth W. Graff, Hockessin, and Albert H. Sherman,  
Wilmington, Del., assignors to ICI America Inc., Wil-  
mington, Del.

No Drawing. Filed Dec. 8, 1969, Ser. No. 883,347  
Int. Cl. C08g 41/00, 43/00

U.S. Cl. 260—239.3 R

7 Claims

**ABSTRACT OF THE DISCLOSURE**

Disclosed are textile treating compositions comprising a novel class of carbamic acid esters containing at least one thermally labile carbamic acid ester group and containing at least one thermally stable carbamic acid ester group derived from a polyoxyethylene ether. The textile treating compositions may be applied to textile materials to improve the physical characteristics thereof; for example, anti-soiling and/or soil release characteristics.

This invention relates to textile treating compositions, to methods of treating textiles, and to textiles having improved physical properties. More particularly, this invention relates to novel carbamic acid esters which are useful for treating textile materials to impart anti-soiling and/or soil release characteristics thereto.

During the past several years, the textile industry has become involved in the durable press treatment of textile materials. Treatment is carried out by impregnating the textile material with an aqueous solution or dispersion of a textile reactive cross-linking durable press agent and then heating the impregnated material for curing. This treatment stabilizes the fibers in the configuration they had in the textile during the curing. Consequently, when a stress is applied to the treated textile and then released, the textile tends to return to the original configuration. This results in a textile material exhibiting durable press properties.

The cross-linking treatment, however, has an adverse effect on the tear strength, hand, soiling, and abrasion resistance properties of the textile material. Thus, the cross-linked textile material, although exhibiting the beneficial characteristics of durable press behavior, has poor abrasion resistance, poor hand, poor texture, and poor soiling properties. It is known that some of the aforementioned properties can be improved by using polyester fibers, alone or in blends with cotton.

Polyester fibers, however, have a propensity to accept and retain oily grime and dirt. Accordingly, when the garment is being worn, soil and/or oily materials accumulate on the garment and settle on the fabric. Once the garment becomes soiled, it is then subjected to a cleaning process for removal of the dirt and/or oily deposits, and only a drycleaning process will successfully clean the garment.

The cleaning process normally employed, however, is washing in a conventional home washing machine by the housewife. During a wash cycle, it is virtually impossible to remove the soil and/or oily stains from the garment and secondly, assuming that the undesirable materials are removed from the garment or a fairly clean garment is being washed, soil remaining in the wash water is redeposited onto the garment prior to the end of the wash cycle. Hence, when the garment is removed from the washing machine and subsequently dried, it has not been properly cleaned. Such a condition, heretofore unavoidable, is quite disadvantageous in that the garment after being worn never again assumes a truly clean appearance, but instead tends to gray and/or yellow due

to the soil and/or oily materials deposited and remaining thereon. Further use and washing of the garment increases the intensity of the gray to the point that ultimately the garment is not acceptable for further wear due to its discoloration.

It is, accordingly, an object of this invention to provide novel textile treating compositions for application to textile materials to impart thereto anti-soiling and/or soil release characteristics to the textile materials and which will adhere to the textile materials through numerous laundering.

It is another object of this invention to provide a process for treating textile material in such a manner that it has anti-soiling and/or soil release characteristics imparted thereto.

It is another object of this invention to provide textile materials having improved anti-soiling and/or soil release properties.

It is an object of this invention to provide a textile treating composition for application to polyester containing textile materials to impart thereto anti-soiling and/or soil release characteristics and which will adhere to the textile materials through numerous laundering.

It is another object of this invention to provide a polyester containing textile material having soil release properties.

It is another object of this invention to provide a process for treating a polyester containing textile material whereby said textile material easily releases soil when contacted with a detergent solution.

It is another object of the present invention to provide a process for treating a polyester containing textile material in such a manner that, after said textile material is soiled and subjected to washing, less soil and grime from the wash water will be redeposited thereon.

It is another object of the present invention to provide a process for treating a textile material in such a manner that it has both a durable press and soil release properties.

It is another object of the present invention to provide a textile treating composition which when applied to textile material imparts thereto both durable press properties and anti-soiling properties.

The foregoing objects and still further objects of this invention are essentially realized by providing a novel class of carbamic acid esters containing at least one thermally labile carbamic acid ester group and containing at least one thermally stable carbamic acid ester group derived from a polyoxyethylene ether as defined below.

The novel carbamic acid esters of the present invention may be prepared by reacting, simultaneously or consecutively in any order, aromatic polyisocyanate, polyoxyethylene ether, and a thermally reversible blocking agent, such as phenol, methyl phenol, dimethyl phenol, trimethyl phenol, ethyl phenol, caprolactam, and mixtures thereof. Thus, the polyisocyanate may be reacted with the blocking agent in such proportions that 1-NCO groups remains and may subsequently be reacted with the polyoxyethylene ether. Alternatively, it is possible to conduct the reaction in the reverse order so that the polyisocyanate is reacted first with the polyoxyethylene ether compound and afterwards with the blocking agent. It is also possible to perform the reaction by mixing all of the reactants in suitable proportions so that the reactions proceed simultaneously.

The amounts of polyoxyethylene ether compound, polyisocyanate, and blocking agent used are selected to assure that the resultant carbamate contains at least one thermally stable carbamate group derived from the polyoxyethylene ether compound, at least one thermally labile carbamate group derived from the blocking agent, and no free isocyanate groups. This may be accomplished

by reacting the polyisocyanate, blocking agent, and polyoxyethylene ether in such proportions that the ratio of mols of blocking agent to NCO groups is less than one and the number of NCO groups is equal to or less than the sum of the hydroxyl groups and mols of blocking agent. Thus, one mol of a polyoxyethylene ether containing two hydroxyl groups and two mols of a diisocyanate may be reacted with two mols of blocking agent whereas one mol of the polyoxyethylene ether and two mols of a triisocyanate may be reacted with four mols of a blocking agent.

The reaction is carried out under conditions which exclude moisture and preferably in the substantial absence of oxygen to minimize discoloration of the resulting carbamic acid ester. Temperatures up to 200° C. may be used. Preferably, the reaction is carried out at 35° C. to 100° C. when caprolactam is used as the blocking agent and at 50° C. to 160° C. when a phenol is used as the blocking agent. The reaction may be conducted in the absence of a solvent or in the presence of a solvent which is inert to isocyanate groups. Illustrative examples of such solvents include cellosolve acetate, acetone, methylethyl ketone, cyclohexanone, chloroform, benzene, perchloroethylene, chlorobenzene, and trifluoroethane. If desired, catalyst such as aliphatic tertiary amines, alkali or alkaline earth metal oxides, carbonates, alcoholates, and phenates, and metal salts of carboxylic acids may be used to facilitate the reaction. If catalyst is used, it should be neutralized after completion of the reaction.

The polyisocyanates which may be used to prepare the carbamic acid ester of this invention are aromatic polyisocyanates; that is, isocyanates containing at least two NCO groups directly attached to carbon atoms of an aromatic ring. Illustrative examples of aromatic polyisocyanates which may be used to prepare the carbamic acid esters of this invention include 2,4-toluene diisocyanate; 2,6-toluene diisocyanate; phenylene diisocyanate; methoxyphenylene 2,4-diisocyanate; diphenylmethane 4,4'-diisocyanate; 3-methyl-diphenylmethane 4,4'-diisocyanate; diphenylether 2,4,4'-trisocyanate; and mixtures thereof. The preferred isocyanate is 2,4-toluene diisocyanate.

The polyoxyethylene ethers which may be used to prepare the carbamic acid esters of this invention are the water-soluble or readily dispersible polyoxyethylene ethers having a molecular weight of at least 6,000, and preferably at least 10,000, and containing at least one aliphatic hydroxyl group, and preferably at least two aliphatic hydroxyl groups, and at least 90% by weight of oxyethylene groups present as polyoxyethylene chains containing at least 60 oxyethylene groups. A preferred class of these polyoxyethylene ethers have a molecular weight of not more than about 100,000 and have two aliphatic primary hydroxyl groups, each of said aliphatic primary hydroxyl groups being directly attached to a polyoxyethylene chain containing at least 6 oxyethylene groups. These polyoxyethylene ethers are well-known compounds and many are commercially available. A particularly preferred class of polyoxyethylene ethers comprises polyoxyethylene glycols having a molecular weight of at least 6,000 and the reaction products of a molar excess of a polyoxyethylene glycol having a molecular weight of at least 3,000 with a compound selected from the group consisting of organic diisocyanates, dicarboxylic acids or anhydrides, and organic diepoxy compounds having two oxirane epoxy groups in which the oxirane oxygen is bonded to adjacent carbon atoms, and preferably to adjacent carbon atoms of a cycloaliphatic ring.

The reaction of the polyoxyethylene glycol with organic diisocyanate may be carried out under reaction conditions conventional in the art for reacting a diisocyanate with a glycol. For example, the reaction may be conducted by heating a mixture of the reactants to a temperature of from 100° C. to 200° C. in the presence or absence of an amine catalyst. The organic diisocyanate may be an aromatic diisocyanate or an aliphatic diisocyanate. Illustrative

of diisocyanates include hexamethylene diisocyanate, toluene diisocyanates, phenylene diisocyanate, diphenylmethane diisocyanates, and methoxyphenylene diisocyanates.

The reaction of the polyoxyethylene glycol with the dicarboxylic acid or anhydride may be carried out under esterification conditions conventional in the art. For example, a mixture of three mols of the glycol and two mols of the acid or anhydride may be heated to a temperature of 150° C. to 200° C. until esterification is essentially complete. The reaction may be conducted in the absence or presence of an acid catalyst, such as toluene-sulfonic acid, or a basic catalyst, such as sodium hydroxide. Illustrative examples of dicarboxylic acids and anhydrides includes succinic acid, maleic acid, terephthalic acid, diglycolic acid, adipic acid, and anhydrides thereof.

The polyoxyethylene ethers prepared by reacting a polyoxyethylene glycol with an organic diepoxy compound are disclosed in United States Pat. Nos. 2,990,396 and 3,182,099. The complete disclosures of these two patents are specifically incorporated into the present application by reference.

The following illustrative examples are given in order that those skilled in the art may better understand the nature and preparation of the carbamic acid esters of the present invention. These examples are set forth solely for the purpose of illustration and any specific enumeration of details contained therein should not be interpreted as expressing limitations of this invention. All parts and percentages are by weight, unless otherwise stated.

#### EXAMPLE 1

188 gms. of phenol is dissolved in about 350 ml. of distilled toluene from which any water has been azeotroped. To this solution are added 348 gms. of 2,4-toluene diisocyanate which is washed into the flask with about 114 ml. of toluene. The mixture is then stirred and refluxed (100–110° C.) under nitrogen for two hours to yield a monophenol-blocked 2,4-toluene diisocyanate solution in toluene. 250 gms. of toluene are added to 374 gms. of Carbowax 6000 (polyoxyethylene glycol of about 6000 molecular weight and sold by Union Carbide), and the mixture is refluxed for about 2 hours to azeotrope about 1 ml. of water. To 50 gms. (0.1 mol reactant) of the above toluene solution of phenol-blocked 2,4-toluene diisocyanate and 100 gms. of dried toluene are added 1.0 gms. of hydrogenated fallow dimethylamine in 5 gms. of toluene. The mixture is then heated to about 80° C., and the above-described Carbowax and toluene solution is added over about a 10-minute period through a steam heated funnel. The stirred mixture is heated at about 80–82° C. for 2 hours. The heat is then removed and the mixture neutralized with 3 gms. of glacial acetic acid washed in with 4.5 gms. toluene, and the toluene vacuum distilled to yield 397 gms. of a viscous, cloudy liquid 1:2:2 Carbowax 600-2,4-toluene diisocyanate-phenol carbamic acid ester product, which hardened to a waxy solid when cold. The product is dispersible in water and soluble in dioxane.

#### EXAMPLE 2

374 gms. of Carbowax 6000 are added to 250 gms. of toluene and the mixture refluxed 1.5 hours to azeotrope 0.5 ml. water to give a hazy viscous product. To this product are added gradually a heated solution (about 80° C.) of 17.5 gms. of 2,4-toluene diisocyanate in 100 gms. of dried toluene. The mixture is heated at 100° C. for 2 hours, and 11.3 gms. of caprolactam in 100 gms. of dried toluene are added to the mixture. The mixture is stirred overnight at about 80° C., and the toluene vacuum stripped to pot temperature of 84° C. to yield 360 gms. of hazy, viscous 1:2:2 condensation product of Carbowax 6000-2,4-toluene diisocyanate-caprolactam. The product is dispersible in water and soluble in dioxane.

## EXAMPLE 3

225 gms. of Carbowax 20M (a polyoxyethylene ether having a molecular weight of 15,000-20,000 and synthesized by reacting about 3 mols of Carbowax 6000 with about 2 mols of diepoxyde. The product is sold by Union Carbide), 17.5 gms. of 2,4-toluene diisocyanate, and 11.3 gms. of caprolactam are reacted in accordance with the process described in Example 2 to give a 1:2:2 addition product of the three reactants. The addition of water to a dioxane solution of the product gives a cloudy solution. A sample of the product is toluene solution diluted with dioxane gave a pale yellow, hazy solution containing 10.5% solids, 12.2% toluene, and 77.3% dioxane.

## EXAMPLE 4

250 gms. of toluene are added to 748 gms. of Carbowax 6000, and the mixture refluxed to about 120° C. for 2 hours to azeotrope 1.0 ml. of water. This solution is then added slowly to 26.2 gms. of 2,4-toluene diisocyanate in 100 gms. of dried toluene over a 10-minute period with stirring. The temperature increases from 58° C. to 81° C. 1.0 gms. of hydrogenated tallow dimethylamine in 5 ml. of toluene is added, and the mixture is heated for about 2 hours at about 80° C. (under a nitrogen blanket). 9.4 gms. of phenol and 50 ml. dried toluene are added and the mixture is stirred overnight at about 80° C. 3.0 gms. of glacial acetic acid is then added and the toluene vacuum stripped from the mixture to yield about 750 gms. of 2:3:2 addition product of Carbowax 6000, toluene diisocyanate, and phenol. The product is soluble in dioxane and dispersible in water.

## EXAMPLE 5

225 gms. of Carbowax 20M are added to 100 of toluene and the water present (about 0.5 ml.) azeotroped off over 1 hour. The toluene is then stripped off under vacuum. 200 ml. ethyl acetate are slowly added at 50° C. of 0.5 gm. of dimethyloctadecylamine and 8.93 gms. of 1:1 2,4-toluene diisocyanate-phenol condensation product (prepared by reacting phenol with toluene diisocyanate for 2 hours at 150° C.) are then added. The mixture is heated at 45° C. with stirring for about 2.5 hours, the catalyst is then neutralized with acetic acid. The solid product is dissolved in warm water to give a slight viscous, milky off-white 10% solution of 1:2:2 condensation product of Carbowax 20M-toluene diisocyanate-phenol.

## EXAMPLE 6

Example 5 is repeated except that 3 times the amount of 1:1 toluene diisocyanate-phenol condensation product is employed. The reaction product is the 1:6:6 condensation product of Carbowax 20M-toluene diisocyanate-phenol.

## EXAMPLE 7

A mixture of 200 ml. of toluene and 225 gms. of Carbowax 20M is azeotroped to remove about 5.0 ml. of water and the toluene distilled under vacuum. 200 ml. ethyl acetate, 17.5 gms. of 2,4-toluene diisocyanate, and 0.5 gm. of dimethyloctadecylamine are added and the mixture heated at about 75° C. with stirring for about 2 hours. 11.3 gms. of caprolactam are added and the temperature is raised to 75° C. and maintained at that temperature with stirring for 12 hours. The product is then cooled, neutralized with glacial acetic acid, and divided into three portions which are respectively dissolved in dioxane, isopropanol, and water. The product is a 1:6:6 condensation product of Carbowax 20M, toluene diisocyanate, and caprolactam.

## EXAMPLE 8

A 1:6:6 condensation product of Carbowax 20M, toluene diisocyanate, and caprolactam is prepared in ac-

cordance with the process of Example 7. The product is divided into three equal portions which are respectively dissolved in Carbitol acetate, propylene glycol, and Ansul 141 for use on textiles.

## EXAMPLE 9

A 1:6:6 condensation product of Carbowax 20M, 2,4-toluene diisocyanate, and caprolactam are prepared in accordance with the process of Example 7 except that Cellosolve acetate is used as a reaction solvent in place of ethyl acetate. The product is separated into three portions which are dissolved in Carbitol acetate, dimethylformamide, and propylene glycol.

## EXAMPLE 10

225 gms. of Carbowax 20M and 50 ml. 1,1,2-trichloroethane are azeotroped to remove any water present and the trichloroethane is distilled off. 185 ml. urethane-grade Cellosolve acetate and 10.4 gms. of caprolactam are added. The mixture is cooled to 45° C., 16.1 gms. of 2,4-toluene diisocyanate is added and the mixture heated at 45-48° C. with stirring for one hour. The condensation product of Carbowax 20M, toluene diisocyanate, and caprolactam is then cooled, divided into three separate portions, and dissolved in Cellosolve acetate, dioxane, and propylene glycol.

## EXAMPLE 11

1125 gms. of Carbowax 20M, 914.8 gms. of urethane-grade Cellosolve acetate, and 230 ml. of 1,1,1-trichloroethane are azeotroped for 45 minutes with collection of 250 ml. of distillate to give an anhydrous product solution. Then, in a separate reaction vessel, 22.6 gms. of caprolactam, 52.2 gms. of 2,4-toluene diisocyanate, and 74.8 gms. of Cellosolve acetate are heated for 4 hours at about 70° C. and the solution cooled. 360.7 gms. of the above Carbowax 20M solution and 24.3 gms. of the toluene diisocyanate-caprolactam product solution are mixed together, heated at about 70° C. with stirring under nitrogen for 3 hours. 89 gms. of propylene glycol are added while heating and stirring are continued. At the end of the reaction, the carbamic acid ester product is diluted to 28% solids concentration with water.

## EXAMPLE 12

The process of Example 11 is modified by heating the 50 final reaction solution only 1 hour at 70° C., then raising the temperature to 90° C. for a further 2 hours reaction and by using about 50% more toluene diisocyanate-caprolactam 1:1 reaction product to give a Carbowax 20M-toluene diisocyanate-caprolactam carbamic acid ester. The product contains 28% solids in a mixture of Cellosolve acetate, propylene glycol, and water.

## EXAMPLE 13

60 To 600 gms. of a polyoxyethylene glycol having an average molecular weight of about 6000, there is added 600 gms. of anhydrous toluene and 2 gms. of boron trifluoride-ether complex (47% boron trifluoride). The mixture is stirred under nitrogen and heated to about 60° C., and 20 gms. of 3,4-epoxy-6-methylcyclohexylmethyl-3,4 - epoxy-6-methylcyclohexanecarboxylate are added. Stirring is continued at about 100° C. for three hours. Then 27 gms. of a 1:1 condensation product of 2,4-toluene diisocyanate and phenol is added and the mixture is stirred for an additional two hours at about 100° C.

## EXAMPLE 14

600 gms. (0.15 mol) of a polyoxyethylene glycol of 75 molecular weight about 4000 is refluxed with 600 ml.

toluene to azeotrope about 1 ml. of water. To the anhydrous solution, there is added 17.4 gms. (0.10 mol) toluene diisocyanate and 1.0 gm. dimethyl octadecylamine and the mixture is heated under nitrogen at about 100° C. for 2 hours with stirring. Then 27 gm. (0.10 mol) of a 1:1 condensation product of 2,4-toluene diisocyanate and phenol is added and the mixture is stirred an additional 2 hours at 100° C.

## EXAMPLE 15

750 gms. (about 0.1 mol) Carbowax 6000 and 6.7 gms. (0.067 mol) succinic anhydride and 0.2 gm. antimony trioxide are stirred under nitrogen and gradually heated to about 200° C. Temperature is maintained at 200° C.-210° C. until esterification is completed. (Acid number reduced to near zero.) The resulting polyester is cooled to 100° C. and diluted with 700 ml. Cellosolve acetate. Then 9.0 gms. (0.033 mol) of a 1:1 2,4-toluene diisocyanate-phenol condensation product is added and the mixture is stirred for two hours at about 100° C.

In accordance with the present invention, carbamic acid esters of the foregoing description may be used to treat textile materials to impart thereto improved physical characteristics such as anti-soiling properties. It has been found that, if the carbamic acid esters are applied to textile materials and then cured by heating the textile material to an elevated temperature, the carbamic acid esters become attached to the textile material so that the improved properties imparted to the textile material will not be removed by subsequent washing. Although this invention is not limited by theoretical considerations, it is believed that the thermally labile carbamate group of the carbamic acid ester decomposes at elevated temperatures to form an aromatic NCO group and free phenol or free caprolactam and that the aromatic NCO group then reacts with the durable press agent, the textile material, and/or other NCO groups to form thermally stable groups.

The carbamic acid esters of the present invention may be advantageously utilized for application to textile materials alone or in combination with a wide variety of chemical treating agents among which are included, for example, durable press compounds, softening compounds, anti-static compounds, emulsifying agents, wetting agents, and numerous other compounds that enhance the physical characteristics of the textile materials. The textile material may be treated with the carbamic acid esters of this invention along with any of the wide variety of chemical treating agents listed above, either simultaneously or separately in any order. A particularly preferred application of the carbamic esters of the present invention is the use of the esters along with a durable press compound. Accordingly, this invention also provides a textile treating composition comprising a durable press resin and a carbamic acid ester.

The amounts of durable press agent and carbamic acid ester present in the textile treating compositions of this invention may vary over a rather wide range and will depend, mainly, on the particular durable press agent and carbamic acid ester selected and on the particular textile material to be treated therewith. In general, the textile treating compositions of this invention may contain from about 50% to 95%, preferably from about 55% to 80%, by weight of the durable press agent and from about 50% to about 5%, preferably from about 45% to 20%, by weight of the carbamate, based on the total weight of durable press agent and carbamate.

Durable press agents useful in the preparation of textile treating compositions in accordance with the present invention include both monomer and polymers which when applied to a textile material and cured under conditions conventional in the art undergo reaction with the textile material and impart durable press and/or wrinkle resistant characteristics to the textile material.

Durable press agents that are preferred when practicing the present invention are the aminoplast resins. These nitrogen containing resins, when applied to textile materials and heated at temperatures at 130° C. to 200° C. in the presence of a catalyst, react with the textile material and become chemically attached thereto. Illustrative examples of the aminoplast resins that may be employed according to the present invention are the ethylene ureas, for example, dimethylol dihydroxy ethylene urea, dimethylol ethylene urea, ethylene urea formaldehyde, and hydroxyethylene urea formaldehyde; urea formaldehyde, for example, propylene urea formaldehyde and dimethylol urea formaldehyde; melamine formaldehyde, for example tetramethylol melamines, and pentamethylol melamines; carbamates, for example, alkyl carbamate formaldehydes; formaldehyde-acrolein condensation products; alkylol amides, for example, methylol formamide and methylol cetamide; acrylamides, for example, n-methylol acrylamide, n-methylol methylacrylamide, and n-methylol-n-methacrylamide; diureas, for example, trimethylol-acetylene diurea and tetramethylol acetylene diurea; triazones, for example, dimethylol-N-ethyl triazine; urons, for example, dimethyloluron and dihydroxydimethyloluron. Mixtures of aminoplast resins may also be used.

Further illustrative examples of durable press agents useful in the preparation of textile treating compositions of this invention include aldehydes, for example, formaldehyde and alpha hydroxy adipaldehyde; epoxides, for example, ethylene glycol diglycidyl ether and vinyl cyclohexene dioxide; ethylene imine derivatives, for example bis aziridinylcarbonyl, and tris(1-aziridinyl)phosphine oxide; chlorohydrins; sulfone derivatives, for example, divinyl sulfone and dihydroxyethyl sulfone; and sulfonium salts, for example, disodium tris(betasulfato ethyl)sulfonium inner salts.

The following are illustrative examples of the textile treating compositions of this invention containing a durable press agent and a carbamic acid ester. It will be appreciated, of course, that additional textile treating compositions of this invention may be prepared by substituting other durable press agents and carbamic acid esters described above for those recited in the following examples. These examples therefore are set forth solely for the purpose of illustration and any specific enumeration of details contained therein should not be interpreted as expressing limitations of this invention. All parts are by weight.

## EXAMPLE 16

|                                    | Parts |
|------------------------------------|-------|
| Carbamate of Example 3             | 36    |
| Dimethylol dihydroxy ethylene urea | 64    |

## EXAMPLE 17

|                                    |    |
|------------------------------------|----|
| Carbamate of Example 5             | 20 |
| Dimethylol dihydroxy ethylene urea | 80 |

## EXAMPLE 18

|                                         |    |
|-----------------------------------------|----|
| Carbamate of Example 1                  | 50 |
| 1,3-dimethylol hexahydro-pyrimidinone-2 | 50 |

## EXAMPLE 19

|                                    |    |
|------------------------------------|----|
| Carbamate of Example 2             | 5  |
| Dimethylol methoxy ethyl carbamate | 95 |

## EXAMPLE 20

|                                     |    |
|-------------------------------------|----|
| Carbamate of Example 3              | 5  |
| Carbamate of Example 4              | 5  |
| Dimethylol-5-hydroxy propylene urea | 90 |

## EXAMPLE 21

|                                                     |    |
|-----------------------------------------------------|----|
| Carbamate of Example 6                              | 25 |
| Disodium tris(β-sulphatoethyl sulfonium) inner salt | 75 |

## EXAMPLE 22

|                                  |    |
|----------------------------------|----|
| Carbamate of Example 7           | 40 |
| Dimethyl hexahydropyrimidinone-2 | 60 |

|                                        |    |
|----------------------------------------|----|
| Carbamate of Example 8                 | 30 |
| Dimethylol dihydroxy ethylene urea     | 35 |
| Dimethylol-5,5-dimethyl propylene urea | 35 |

In accordance with the present invention, the above described textile treating compositions containing a durable press agent and a carbamic acid ester may be used to treat textile materials to impart thereto physical characteristics such as durable press, wrinkle resistance, tear and tensile strength, hand, abrasion resistance, soil release properties, and anti-redeposition properties. It has been found that if the textile treating compositions of this invention are applied to textile material and the treated textile material heated to an elevated temperature, the durable press agents and the carbamic acid ester will react so that the improved properties imparted to the textile material will not be removed by subsequent washing.

The textile resins catalyst for the durable press agent may be any of the acid or latent acid catalysts which are conventionally used in the art to facilitate reaction of durable press agents with textile material. By latent acid catalyst is meant a substance which develops acidity during the curing step. Particularly suitable catalysts include metal salts of strong acids, for example, magnesium chloride, magnesium sulfate, zinc nitrate, and aluminum sulfate; ammonium salts, for example, ammonium chloride, ammonium dihydrogen phosphate, and ammonium thiocyanate; amine salts, for example, triethyl amine hydrochloride and triethanolamine hydrochloride.

The amount of curing catalyst used for the durable press agent depends on the nature of the durable press agent, catalyst and on the curing temperature and curing time. In general, satisfactory results may be obtained by using from about 1% to about 50%, preferably from about 10% to about 35%, by weight of the catalyst based on the weight of durable press agent. The amount of catalyst to be utilized is that conventionally used in activating the reaction between durable press resins and active hydrogen atoms present in the textile materials to be treated therewith.

The textile treating compositions of this invention may be applied to textile materials from an aqueous medium, an organic solvent, or an emulsion of water and organic solvent. Illustrative examples of organic solvents which may be used include isopropanol, 1,1,1-trichloroethane, 1,1,2-trichloroethane, perchloroethylene, carbon tetrachloride, chloroform, pentachloroethane, and a dichlorobenzene. Illustrative examples of surfactants which may be used to emulsify the carbamic acid ester in organic solvents include polyoxyethylene(25) castor oil, isopropylamine dodecylbenzene sulfonate, diethyl sulfate quaternary of polyoxyethylene(20)hydrogenated tallow amine and polyoxyethylene(10) nonyl phenol.

Textile materials may be treated with the bath containing a textile treating composition of this invention by any suitable means, such as by immersion therein or by spraying. In the immersion method of application, the textile material may either be run through a padding machine where the textile material is first dipped into the bath and then squeezed, or the textile materials may be dipped into the bath and the excess liquid extracted by centrifugation. In the spraying method of application, the textile materials are simply sprayed with the bath and dried by any suitable means. The carbamic acid ester, durable press agent, and textile resin catalyst may be applied simultaneously or from separate baths. The catalyst for the durable press agent may be applied with the durable press agent and/or carbamic acid ester or from a separate bath.

The amount of carbamic acid ester applied to the textile material may vary from about 0.1% to about 10%, preferably from about 0.5% to about 5%, by weight based on the dry weight of the textile material.

It is necessary to subject the textile material having the carbamic acid ester thereon to an elevated temperature in order to initiate and curing reaction between the carbamic acid ester and the textile material. The particular temperature used and the duration of the heating step depends on the nature of the textile material used and on the particular carbamic acid ester used. In each situation, however, the temperature and heating time is that necessary to sufficiently cause reaction of the carbamic acid ester with the textile material. Generally, the heat cure may be effected at temperatures from about 100° F. to about 350° F. and in periods of time ranging from about 40 to about 60 minutes at the lower temperature to about 0.5 to 10 minutes at the higher temperature. The preferred temperature is from about 300 to 350° F.

Textile materials which may be treated with the textile compositions of this invention include any textile material conventionally treated in the art with durable press and/or antisoiling agents; for example, textile material comprising cellulose or modified cellulose such as cotton, rayon, linen, and mixtures thereof; textile material containing non-cellulosics such as polyesters, nylon, acrylics, and mixtures thereof; and textile materials comprising a blend of cellulosic materials and non-cellulosic materials. The textile materials may be in the form of filaments, fibers, threads and yarns or in the form of woven, non-woven, knit, or otherwise formed fabrics, sheets, and cloths. The preferred textile materials are polyester fabric and cotton/polyester blends.

The following examples are illustrative of the application of textile treating compositions of this invention to textile materials. These examples are set forth solely for the purpose of illustration and any specific enumeration of details contained therein should not be interpreted as expressing limitations of this invention. All parts and percentages are by weight, unless otherwise stated.

The following procedures and abbreviations are used throughout the following examples:

Soil redeposition is determined versus untreated fabric. About 16 ml. of a standard stock soiling mixture containing 38% peat moss, 17% Corson's Home-Crete (sand mix), 17% kaolin clay (Peerless clay #2), 17% silica (200 mesh), 1.75% Molacco furnace black, 0.5% red iron oxide N-1860, and 8.75% Nujol is diluted to one liter with hot tap water, 6 x 6-inch test swatches of the above treated fabrics are immersed in 200 ml. of the soil solution, the cloth agitated in the soil solution about 30 minutes at about 140° F. along with duplicated samples in 1% Tide detergent solutions, the swatches removed, rinsed thoroughly in cool tap water, tumble dried in a standard automatic clothes drier at about 160° F. and the soiled samples rated against the control samples. After washing in Tide and hot water, the samples were rated:

EOS—Excessive retained oil and solid soil

S—Retained solid soil

SS—Slight retained solid soil

NR—No retention of oil or solid soil

Soil release ratings of the treated textiles were determined by the Deering Milliken Research Corporation stain release procedure. Four drops of Gulf transmission fluid is allowed to fall on a glass surface, after 15 seconds a specimen of test cloth is placed on the oil, a sheet of polyethylene is placed over the test cloth, a standard 8-pound weight placed on the polyethylene over the oil spot, the weight, polyethylene, and cloth are removed after 30 seconds, the test cloth placed between two paper towels, the weight applied for 30 seconds, the test cloth washed once, and rated visually for soil release versus a photographic standard. Soil release ratings are from 5.0, "no soil retained," to 1.0, "no soil released."

The following laboratory laundering procedure is used for all washes. The samples and at least 3 pounds of 8-oz. fabric in 36 x 36-inch pieces are loaded into a standard automatic washer, about 46 grams of Tide deter-

gent added, about 120° F. water run in, and the samples washed on a 12-minute wash cycle. After the required number of wash cycles, the samples and the cloth are dried about 45 minutes at about 160° F. and pressed with a hand iron. Pressing is omitted when a durable press finish has been applied to the samples in addition to the carbamate.

In Examples 24 through 27, textile treating pad baths having the indicated compositions are padded onto 100% polyester fabrics at 80% wet pickup on the Butterworth pad. The treated fabrics are dried at 212° F. for 3 minutes. Samples of each treated fabric are cured at 250° F. for 3 minutes, 325° F. for 12 minutes, and 400° F. for 10 minutes, respectively, and conditioned overnight at room temperature prior to testing. The results are shown in Table I.

TABLE I

| Example Number     | Bath | Soil redeposition at— |         |         | Soil release ratings at— |         |         |
|--------------------|------|-----------------------|---------|---------|--------------------------|---------|---------|
|                    |      | 250° F.               | 325° F. | 400° F. | 250° F.                  | 325° F. | 400° F. |
| Untreated fabrics. |      | EOS                   | EOS     | EOS     | 4                        | 3       | 3       |
| 24                 | (1)  | SS                    | SS      | EOS     | 5                        | 5       | 4       |
| 25                 | (2)  | SS                    | S       | S       | 4                        | 5       | 4       |
| 26                 | (3)  | SS                    | SS      | S       | 5                        | 5       | 4       |
| 27                 | (4)  | SS                    | SS      | S       | 4                        | 4       | 4       |

<sup>1</sup> 1.35 parts of the carbamate of Example 1 and 98.65 parts of water.

<sup>2</sup> 1.35 parts of the carbamate of Example 2, 0.07 parts of dimethylstearylamine acetate, and 98.58 parts of water.

<sup>3</sup> 12.86 parts of the carbamate solution of Example 3, 0.07 part of dimethylstearylamine acetate, 3.21 parts of isopropanol, and 83.86 parts of water.

<sup>4</sup> 1.35 parts of the carbamate of Example 4 and 98.65 parts of water.

In Examples 28 and 29, textile treating baths having the indicated compositions are padded onto 65:35 polyester cotton blend fabrics at 80% wet pickup on the Butterworth pad. The treated fabrics are dried at 212° F. for 3 minutes and cured at 325° F. for 10 minutes. The test results are shown in Table II.

TABLE II

| Example Number | Bath | Soil redeposition | Soil release |
|----------------|------|-------------------|--------------|
| Control        | (1)  | EOS               | 2            |
| 28             | (2)  | S                 | 4            |
| 29             | (3)  | S                 | 3            |

<sup>1</sup> 10.8 parts of dihydroxy dimethylol ethylene urea, 1.35 parts of zinc nitrate hexahydrate, and 87.85 parts of water.

<sup>2</sup> 9.53 parts of the product of Example 3 (1 part carbamate), 5 parts of zinc nitrate hexahydrate, and 85.47 parts of water.

<sup>3</sup> 1 part of the carbamate of Example 4, 10.8 parts of dihydroxy dimethylol ethylene urea, 1.35 parts of zinc nitrate hexahydrate, and 86.85 parts of water.

In Examples 30, 31, 32, and 33, textile treating baths containing 20 parts of 45% aqueous solution of dihydroxy dimethylol ethylene urea, 1.5 parts of 65% aqueous solution of magnesium dichloride hexahydrate, the indicated amounts of carbamate, and water to 100 parts are made up and applied to 65:35 polyester-cotton blend fabrics at 70% wet pickup on the Butterworth pad. The treated fabrics are dried at 225° F. for 3 minutes and cured at 325° F. for 10 minutes. Half of the treated fabrics are washed 5 times with detergent in hot water. All fabrics are conditioned overnight at 65% relative humidity and 72° F. prior to testing. Soil release ratings are made after immersing the fabrics in soiling solution prior to laundering and again after applying the soiling solution after 5 launderings. Test results are given in Table III.

TABLE III

| Example Number | Carba-mate | Redeposition ratings after— |          | Soil release ratings after— |          |
|----------------|------------|-----------------------------|----------|-----------------------------|----------|
|                |            | 0 washes                    | 5 washes | 0 washes                    | 5 washes |
| Control        | (1)        | EOS                         | EOS      | 1                           | 1        |
| Do             | (2)        | EOS                         | EOS      | 1                           | 1        |
| 30             | (3)        | NR                          | SS       | 3                           | 3.5      |
| 31             | (4)        | NR                          | S        | 2.5                         | 3        |
| 32             | (5)        | NR                          | SS       | 3                           | 3        |
| 33             | (6)        | NR                          | NR       | 4                           | 4        |

<sup>1</sup> Untreated fabric.

<sup>2</sup> Fabric treated with bath containing 9 parts of dihydroxy dimethylol ethylene urea, 1 part of magnesium dichloride hexahydrate, and 90 parts of water.

<sup>3</sup> 50 parts of a 10% aqueous solution of the carbamate of Example 5.

<sup>4</sup> 18 parts of a 28% solution of the carbamate of Example 6 in dioxane and ethyl acetate.

<sup>5</sup> 18 parts of a 28% solution of the carbamate of Example 6 in water and ethyl acetate.

<sup>6</sup> 14 parts of a 32.7% solution of the carbamate of Example 7 in ethyl acetate and isopropanol.

In Examples 34 and 35, textile treating baths having the indicated compositions are applied to 100% polyester fabrics at 80% wet pickup on the Butterworth pad. The treated fabric samples are dried at 225° F. for 3 minutes and cured at 375° F. for 30 seconds. Half of the samples are washed 10 times with Tide in hot water. All samples are conditioned overnight prior to testing. The test results are shown in Table IV.

TABLE IV

| Example Number   | Bath | Redeposition ratings after— |             | Soil release ratings after— |           |
|------------------|------|-----------------------------|-------------|-----------------------------|-----------|
|                  |      | 0 washes                    | 5-10 washes | 0 washes                    | 10 washes |
| Untreated fabric |      | EOS                         | EOS         | 1                           | 1         |
| 34               | (1)  | NR                          | NR          | 4.5                         | 4.5       |
| 35               | (2)  | NR                          | NR          | 5                           | 5         |

<sup>1</sup> 5 parts of a 28% solution of the carbamate of Example 9 in Cellosolve acetate and propylene glycol plus 95 parts of water.

<sup>2</sup> 5 parts of a 28% solution of the carbamate of Example 8 in ethyl acetate and propylene glycol plus 95 parts of the water.

In Examples 36 and 37, textile treating baths containing 20 parts of 50% aqueous solution of dihydroxy dimethylol ethylene urea, 5 parts of a 65% aqueous solution of magnesium chloride hexahydrate, 18 parts of the indicated carbamate solution, and 57 parts of water are applied to 65:35 polyester-cotton blend fabrics at 70% wet pickup on the Butterworth pad. The treated fabrics are dried at 225° F. for 3 minutes and cured at 325° F. for 10 minutes. Half of the treated fabrics are washed 10 times with detergent in hot water. All fabrics are conditioned overnight at 65% relative humidity and 72° F. prior to testing. Soil release ratings are made after immersing the fabrics in soiling solution prior to laundering and again after applying the soiling solution after 10 launderings. Test results are shown in Table V.

TABLE V

| Example Number | Carba-mate solution | Redeposition ratings after— |           | Soil release ratings after— |           |
|----------------|---------------------|-----------------------------|-----------|-----------------------------|-----------|
|                |                     | 0 washes                    | 10 washes | 0 washes                    | 10 washes |
| Control        | (1)                 | SS                          | SS        | 3                           | 2         |
| Do             | (2)                 | EOS                         | EOS       | 2                           | 2         |
| 36             | (3)                 | NR                          | SS        | 4.5                         | 3         |
| 37             | (4)                 | NR                          | SS        | 4.5                         | 4         |

<sup>1</sup> Untreated fabric.

<sup>2</sup> Fabric treated with bath containing 20 parts of 50% aqueous solution of dihydroxy dimethylol ethylene urea, 5 parts of a 65% aqueous solution of magnesium chloride hexahydrate and 75 parts of water.

<sup>3</sup> 28% solution of the carbamate of Example 9 dissolved in Cellosolve acetate and propylene glycol.

<sup>4</sup> 28% solution of the carbamate of Example 8 dissolved in ethyl acetate and propylene glycol.

In Example 38, a textile treating bath is prepared containing 1.45 parts of the carbamate of Example 10, 1.05 parts of Cellosolve acetate, 2.5 parts of propylene glycol and 95 parts of water. The bath is padded onto 100% polyester fabric at 80% wet pickup. The treated fabric samples are dried at 225° F. for 3 minutes and cured at

## 13

375° F. for 30 seconds. Half of the samples are washed 5 times with Tide in hot water. All samples are conditioned overnight prior to testing. The test results are shown in Table VI.

TABLE VI

| Example Number        | Redeposition ratings after— |          | Soil release ratings after— |          |
|-----------------------|-----------------------------|----------|-----------------------------|----------|
|                       | 0 washes                    | 5 washes | 0 washes                    | 5 washes |
| Untreated fabric..... | EOS                         | EOS      | 1.7                         | 1.5      |
| Example 38.....       | NR                          | NR       | 4.0                         | 3.5      |

In Example 39, a textile treating bath containing 9 parts of dihydroxy dimethylol ethylene urea, 3.2 parts of magnesium chloride hexahydrate, 5.8 parts of the carbamate of Example 10, 4.2 parts of Cellosolve acetate, 10 parts of propylene glycol, and 67.8 parts of water is applied to 65:35 polyester-cotton blend fabric at 75% wet pickup. The treated fabrics are dried at 225° F. for 3 minutes and cured at 325° F. for 10 minutes. Half of the treated fabrics are washed 5 times with detergent in hot water. All treated fabrics are conditioned overnight at 65% relative humidity and 72° F. prior to testing. Soil release ratings are made after immersing the fabrics in soiling solution prior to laundering and again after applying the soiling solution after 5 launderings to test results as shown in Table VII.

TABLE VII

| Example number             | Redeposition ratings after— |          | Soil release ratings after— |          |
|----------------------------|-----------------------------|----------|-----------------------------|----------|
|                            | 0 washes                    | 5 washes | 0 washes                    | 5 washes |
| Control <sup>1</sup> ..... | EOS                         | EOS      | 2.0                         | 1.5      |
| Do <sup>2</sup> .....      | EOS                         | EOS      | 1.5                         | 1.3      |
| Example 39.....            | SS                          | NR       | 3.5                         | 3.3      |

<sup>1</sup> Untreated fabric.

<sup>2</sup> Fabric treated with a bath containing 9 parts of dihydroxy dimethylol ethylene urea, 3.2 parts of magnesium chloride hexahydrate, 4.2 parts of Cellosolve acetate, 10 parts of propylene glycol, and 73.6 parts of water.

In Examples 40 and 41, textile treating baths containing 20 parts of a 45% aqueous solution of dihydroxy dimethylol ethylene urea, 3.3 parts of magnesium chloride hexahydrate, 20 parts of the indicated carbamate solution, and sufficient water to make 100 parts are padded on 50:50 polyester-cotton blend fabrics at 70% wet pickup. The treated fabrics are dried at 225° F. for 3 minutes and cured at 325° F. for 10 minutes. Half of the treated fabrics are washed 5 times with detergent and hot water. All fabrics are conditioned overnight at 65% relative humidity and 72° F. prior to testing. Soil release ratings are made after immersing the fabrics in soiling solution prior to laundering and again after applying the soiling solution after 5 launderings. Test results are given in Table VIII.

TABLE VIII

| Example number | Carba-<br>mate<br>solution | Redeposition<br>ratings after— |             | Soil release<br>ratings after— |             |
|----------------|----------------------------|--------------------------------|-------------|--------------------------------|-------------|
|                |                            | 0<br>washes                    | 5<br>washes | 0<br>washes                    | 5<br>washes |
| Control.....   | ( <sup>1</sup> ) S         | NR                             | 2.0         | 2.3                            |             |
| Do.....        | ( <sup>2</sup> ) EOS       | EOS                            | 1.0         | 2.3                            |             |
| 40.....        | ( <sup>3</sup> ) SS        | SS                             | 3.5         | 3.5                            |             |
| 41.....        | ( <sup>4</sup> ) SS        | SS                             | 3.0         | 1.8                            |             |

<sup>1</sup> Untreated fabric.

<sup>2</sup> Fabric treated with a bath containing 20 parts of 45% aqueous solution of dihydroxy dimethylol ethylene urea 3.3 parts of magnesium chloride hexahydrate and sufficient water to make 100 parts of bath.

<sup>3</sup> Carbamate solution of Example 11.

<sup>4</sup> Carbamate solution of Example 12.

Although this invention has been described with reference to specific organic polyisocyanates, blocking agents, polyethylene glycol ethers, linear polyurethanes, dicarboxylic acids and anhydrides thereof, cycloaliphatic di-epoxy compounds, durable press agents, textile resin catalyst, solvents, and textile materials and to specific processes and method steps, it will be apparent that other equivalent materials may be substituted for those specific

## 14

cally described and the method steps and types of processes may be altered, all within the spirit and scope of this invention.

Having described the invention, what is desired to be secured by Letters Patent is:

1. A composition of matter which consists essentially of the reaction product of

(a) an organic aromatic polyisocyanate containing at least 2 NCO groups directly attached to carbon atoms of an aromatic ring,

(b) a thermally reversible blocking agent selected from the group consisting of caprolactam, phenol, lower alkyl substituted phenols containing from 1 to 2 alkyl groups, and mixtures thereof and

(c) a polyoxyethylene ether having a molecular weight of at least 6,000, and containing at least two aliphatic hydroxyl groups and at least 90% by weight of oxyethylene groups present as polyoxyethylene chains containing at least 60 oxyethylene groups, said reaction being carried out at a temperature from ambient temperature to 200° C. and the amounts of organic aromatic polyisocyanate, thermally reversible blocking agent, and polyoxyethylene ether are selected to furnish a ratio of mols of blocking agent to NCO groups present in the aromatic polyisocyanate of less than 1 and a number of NCO groups of not more than the sum of the hydroxyl groups and mols of blocking agent.

2. A composition of claim 1 wherein the thermally reversing blocking agent is selected from the group consisting of caprolactam, phenol, methylphenol, dimethylphenol, trimethylphenol, ethylphenol, and mixtures thereof.

3. A composition of claim 2 wherein the polyoxyethylene ether (c) is a polyoxyethylene glycol having a molecular weight of at least 6,000.

4. A composition of claim 2 wherein the polyoxyethylene ether (c) comprises the reaction product of a diisocyanate with a molar excess of a polyoxyethylene glycol having a molecular weight of at least 3,000.

5. A composition of claim 2 wherein the polyoxyethylene ether (c) comprises the reaction product of a dicarboxylic acid or anhydride with a molar excess of a polyethylene glycol having a molecular weight of at least 3,000.

6. A composition of claim 2 wherein the polyoxyethylene ether (c) comprises the reaction product of an organic diepoxy compound having two oxirane epoxy groups in which the oxirane oxygen is bonded to adjacent carbon atoms with a molar excess of a polyethylene glycol having a molecular weight of at least 3,000.

7. A composition of claim 1 wherein the organic aromatic polyisocyanate is selected from the group consisting of 2,4-toluene diisocyanate; 2,6-toluene diisocyanate; phenylene diisocyanate; methoxyphenylene 2,4-diisocyanate; diphenylmethane 4,4'-diisocyanate; 3-methyl-diphenylmethane 4,4'-diisocyanate; diphenylether 2,4,4'-triisocyanate; and mixtures thereof.

## References Cited

## UNITED STATES PATENTS

3,454,621 '7/1969 Engel ----- 260—471 C  
3,483,189 12/1969 Brotherton et al. 260—239.3 R

## FOREIGN PATENTS

701,711 12/1953 Great Britain 260—239.3 R  
891,009 3/1962 Great Britain 260—479 C

HENRY R. JILES, Primary Examiner

R. T. BOND, Assistant Examiner

## U.S. CL. X.R.

260—77.5 AT, 77.5 TB, 468 C, 468 E, 471 C, 479 C,  
482 B, 482 C; 8—115.5, 116.2, 127.6, 129

UNITED STATES PATENT OFFICE  
CERTIFICATE OF CORRECTION

Patent No. 3,738,981 Dated June 12, 1973  
Inventor(s) Kenneth W. Graff and Albert H. Sherman

It is certified that error appears in the above-identified patent  
and that said Letters Patent are hereby corrected as shown below:

Column 3, line 39, "4,,4'-diisocyanate;" should read  
-- 4,4'-diisocyanate; --.  
line 55, "6" should read -- 60 --.  
Column 5, line 12, "is" should read -- in --.  
line 35, after "100" insert -- ml. --.  
line 38, delete "of".  
line 58, "5.0" should read -- 0.5 --.  
Column 10, line 48, "duplicated" should read -- duplicate --.  
Column 12, line 38, after "of" delete "the".  
line 44, "polyester-cottorn" should read  
-- polyester-cotton --.

Signed and sealed this 8th day of January 1974.

(SEAL)  
Attest:

EDWARD M. FLETCHER, JR.  
Attesting Officer

RENE D. TEGTMEYER  
Acting Commissioner of Patents